

R. D. HEACOX,  
METHOD OF REPAIRING SCORED CYLINDERS.  
APPLICATION FILED MAR. 18, 1921.

1,385,334.

Patented July 19, 1921.

*Fig. 1.*



*Fig. 4.*



*Fig. 2.*



*Fig. 5.*



*Fig. 3.*



*Fig. 6.*



ROSS D. HEACOX

INVENTOR.

BY

Mason Fenwick & Lawrence  
ATTORNEY.

# UNITED STATES PATENT OFFICE.

ROSS D. HEACOX, OF WASHINGTON, DISTRICT OF COLUMBIA.

## METHOD OF REPAIRING SCORED CYLINDERS.

1,385,334.

Specification of Letters Patent. Patented July 19, 1921.

Application filed March 18, 1921. Serial No. 453,502.

To all whom it may concern:

Be it known that I, Ross D. HEACOX, a citizen of the United States, residing at Washington, in the District of Columbia, 5 have invented certain new and useful Improvements in Methods of Repairing Scored Cylinders; and I do hereby declare the following to be a full, clear, and exact description of the invention, such as will enable others, skilled in the art to which it appertains 10 to make and use the same.

This invention relates to a method for repairing scored metal objects.

The main object of the invention is to provide a method by which scored engine cylinders may be simply, efficiently and economically repaired without the necessity for regrinding; which process will result in a practical and substantially permanent 15 remedy.

The invention consists in the novel steps, processes, methods and materials hereinafter more particularly described and claimed.

One sheet of drawings accompanies this 25 specification as part thereof, in which like reference characters indicate similar parts throughout.

The figures are all fragmentary transverse sections of an engine cylinder.

30 Figure 1 illustrates the cylinder with two narrow scores;

Fig. 2 illustrates the scores of Fig. 1 after they have been preliminarily cleaned out and prepared and filled with an alloy metal 35 preliminary to scraping;

Fig. 3 shows the cylinder of Fig. 1 after the process has been completed and the surplus alloy metal has been scraped off to the true contour of the cylinder;

40 Fig. 4 illustrates a broad, shallow score;

Fig. 5 illustrates a broad, shallow score cleaned out and double dove-tailed and filled with an alloy metal, and

Fig. 6 shows the final step with the broad 45 score filled and finished.

It is a common occurrence in the use of explosive engines for the wrist pins to break or work loose so as to come in contact with and score the cylinder wall. Such scores may 50 be eliminated if the cylinder wall is sufficiently thick by regrinding the cylinder, but this necessarily weakens the cylinder throughout, requires expensive machinery and the removal of the engine.

55 In accordance with the present invention, the scores in the cylinder are first cleaned

out with suitable scraping tools until they have smooth bottoms 4 and undercut or dove-tailed sides 3-3, as illustrated in Fig. 2. This is ordinarily sufficient in the case 60 of narrow scores such as Fig. 2, but where the scores are broad as 2', it is desirable to further deepen the score centrally and provide a further lower bottom 4' and supplementary undercut sides 3', making a fur- 65 ther dove-tailed seat in the middle of the score as illustrated in Fig. 5.

When the scores have been thus cleaned out and shaped, a suitable flux such as "killed spirits" or muriate of zinc is applied 70 and the surface is tinned over throughout with the alloy or solder with which the score is to be filled. The score is then completely filled with a hard solder which has the characteristic of expanding upon solidifying. 75 Antimony in suitable proportions is known to produce this effect in alloy solders and it may be generally stated that any hard solder having this quality is adaptable for use in this process. One formula for such a solder, which experiments indicate is particu- 80 larly suitable, consists of 50 per cent. tin, 30 per cent. lead, 15 per cent. antimony and 5 per cent. copper. This alloy has a melting point between 450°-480° F. 85

The scores are well filled with this solder so that its upper surface extends slightly above the normal surface of the cylinder. A scraper gaged accurately to the contour of the cylinder is then used to remove the sur- 90 plus alloy metal and bring its surface to the true contour of the cylinder. An adjustable scraper peculiarly adapted to this operation is described in my co-pending application, Serial No. 452,868, Mar. 16, 1921. 95

It will be noted that in addition to the gripping surfaces provided by the undercut walls of the scores described above, the alloy metal will be further secured to the cylinder wall by reason of the natural porosity of the 100 cast iron. Experiments indicate that the highly fluid molten alloy metal penetrates the pores of the iron and by reason of its quality of expanding in cooling grasps the iron and roots the insert to its place. 105

Having thus fully described my invention, I claim:

1. A process of repairing scored cylinders which consists in cleaning and fluxing the scores and then soldering therein a hard solder having the property of expanding on 110 cooling.

- 2
- 2. The process of repairing scored cylinders which consists in cleaning and fluxing the score and soldering therein a hard solder comprising tin, lead, antimony and copper.
  - 5 3. The process of repairing scored cylinders which consists in scraping out the score to provide a seat having undercut side walls,

filling said seat with a solder having the property of expanding on cooling and scraping the surplus solder away to the true contour of the cylinder wall. 10

In testimony whereof I affix my signature.

ROSS D. HEACOX.